

N. V. HYBINETTE.  
 PROCESS OF REFINING LEADY MATTE.  
 APPLICATION FILED JAN. 25, 1915.

1,175,266.

Patented Mar. 14, 1916.



**Fig.2.**



**Fig.3.**



Witnesses:

B. Dommers  
 E. Leckert.

Inventor.

Noak Victor Hybinette,  
 By *Henry M. Jr.* Atty.

# UNITED STATES PATENT OFFICE.

NOAK VICTOR HYBINETTE, OF CHRISTIANIA, NORWAY.

## PROCESS OF REFINING LEADY MATTE.

1,175,266.

Specification of Letters Patent. Patented Mar. 14, 1916.

Application filed January 25, 1915. Serial No. 4,255.

*To all whom it may concern:*

Be it known that I, NOAK VICTOR HYBINETTE, a subject of the King of Norway, residing at Christiania, Norway, have invented certain new and useful Improvements in Processes of Refining Leady Matte; and I do hereby declare the following to be a full, clear, and exact description of the invention, such as will enable others skilled in the art to which it appertains to make and use the same, reference being had to the accompanying drawings, and to letters or figures of reference marked thereon, which form a part of this specification.

15 My invention relates to the treating of so called leady matte, that is to say copper matte containing more or less, generally a considerable amount of lead. It is well known that there are several difficulties connected with the treating of this material, and that the processes hitherto known for refining the same not only are very expensive and requiring very great plants, but also result in the loss of lead, the usual 20 way of refining such matte being to blow off the lead together with impurities in a converter whereby it is necessary to treat the flue dust in an elaborate process for extracting the lead.

25 My invention consists in a process, in which I obtain the lead and with the lead also the precious metals and other elements in the matte directly from the molten matte by way of a contact action, in which pure copper causes the separation of the lead. By causing this action to be effected on the counter current principle, I am able to carry out the process in such way that I can produce either pure copper or copper refined to 30 such degreee, that the complete refinement may easily be performed electrolytically and on the other hand I obtain metallic lead which may easily be purified, thereby obtaining silver, arsenic and other valuable 35 products.

In the following I shall explain my invention reference being thereby had to the annexed drawing, in which—

40 Figure 1 is a diagram illustrating one form of apparatus for carrying out the process, and Fig. 2 is a diagrammatic horizontal section on line 3—3 of Fig. 3, of a continuously operating furnace, and Fig. 3 is a vertical section on line 2—2 of Fig. 2.

45 According to my process I melt the leady matte in a suitable furnace as for instance

A. The molten matte is taken over to one or more furnaces, in which the matte is held at the suitable temperature, and in which the lead is separated by forming a bottom of 50 metallic lead in the said furnace or furnaces. In the diagram Fig. 1 is shown a series of three furnaces B, C, D. The matte comes first to the furnace B, then to furnace C and lastly to furnace D. From the latter it is 55 brought to a Bessemer converter E. When it is introduced in the converter it is or may be practically free from lead. In the Bessemer converter the matte is treated in the usual way to obtain pure copper. Part 60 of this pure copper is caused to pass the furnaces B, C, D in a direction opposite to the direction in which the matte passed the said furnaces. The effect of the pure copper coming into contact with matte containing lead is that a bottom of metallic 65 lead is separated, and as the matte and the copper pass the separating furnace or furnaces in opposite directions, the matte will successively lose its contents of lead and 70 take up the equivalent amount of copper from the bottom. Together with the lead bottom precious metals as silver, gold and also arsenic, antimony and other elements 75 will be separated. If a number of separating furnaces is used as indicated in the diagram, these may be tilting furnaces of the crucible type and the materials in the furnaces may be passed over from one to another by way of a ladle.

80 Referring to the diagram, Fig. 1, a represents the furnace or equivalent for melting the matte. This matte, as indicated by the arrow, is transferred to the first crucible b or equivalent by a ladle or otherwise, while 85 lead is tapped off from the bottom. The upper layer of matte in crucible b is ladled out into crucible c and the bottom layer of more refined matte from crucible c is transferred into crucible b as indicated by the 90 arrow m. The upper layer in crucible c is transferred to the converter. This diagram presupposes a ladling operation, and the matte may be considered as treated in stages, but these stages may be so merged into one 95 another as to make the process substantially continuous, by the use of a single separating furnace in the place of the crucibles.

100 If only a single separating furnace is used this may be in the form of a long furnace V as shown in plan view in Fig. 2. Such furnace may be provided with stag-

gered deflecting walls *W* placed alternately on one and on the other side wall of the furnace, so that the materials are caused to pass through the furnace in a curved line, 5 the matte being introduced at one end and the copper at the other.

From an inspection of Figs. 2 and 3 it will be seen that the matte is introduced at the right hand end of such a furnace to the 10 upper layer of the molten bath, and crude lead drawn off at the bottom at said end. Copper is introduced at the opposite end to the upper layer of the molten bath, and refined matte, *i. e.* substantially copper sulfid, 15 withdrawn from below the molten surface. Referring to Fig. 2, the matte may be considered as taking the course of the full arrows, as indicated by the arrow *y* into crucible *d*, while the lower layer in crucible *d* is transferred, as indicated by the arrow *n* 20 to crucible *c*. The top layer of the last crucible, which is refined matte, is transferred to the converter *e*, and is substantially copper sulfid. The sulfur is removed 25 as is customary in bessemerizing copper matte, and copper discharged. Some of the bessemerized matte or copper discharged from the converter is transferred to the last crucible. The number of crucibles between 30 the melting furnace *a* and converter *e* will depend upon the character of the matte handled. It will thus be seen that the contents of the crucibles increase in copper content toward the converter *e* while the 35 lead content decreases, practically pure copper sulfid being taken from the top layer of the crucible, and lead containing other reduced metals from the first crucible *a*, the matte from the melting furnace *a* traveling counter to the copper introduced from the converter *e*, the matte taking the course indicated by the full arrows, and the copper the course of the dotted arrows.

Other kinds of apparatus than above indicated may of course be used for carrying out the process.

What I claim is:

1. The method of refining copper matte containing sulfids of lead and other metals, 50 which comprises melting the matte, refining

same by adding bessemerized matte to the molten matte, bessemerizing the refined matte and drawing off the crude lead resulting from the refining step.

2. The method of refining matte, which 55 comprises freeing the metal constituent of a maintained bath of matte having the greatest affinity for sulfur from its combined sulfur and adding a portion of resulting metal to a fresh quantity of molten 60 matte, thereby increasing in the matte its content of said metal and causing the reduction of the other sulfid contents to metal.

3. The method of refining copper matte containing sulfids of lead and other metals, 65 which comprises progressing matte in molten condition through successive receptacles, bessemerizing the matte from the last receptacle, returning bessemerized matte to the last receptacle, and progressing separated 70 constituents through the receptacles counter to the aforesaid progression of the matte.

4. The method of refining copper matte containing sulfids of lead and other metals, 75 which comprises maintaining a molten bath of matte, constraining the flow of metal from one end of the bath to the other, introducing molten matte and withdrawing lead at one end of said bath at different levels, and introducing bessemerized matte 80 and withdrawing refined matte at the other end of said bath at different levels.

5. The method of refining mixed sulfids, 85 which comprises maintaining a long molten bath of matte, retarding the flow of the bath from one end to the other, introducing molten sulfids and also withdrawing a metal at one end of said bath but at different levels, introducing a reduced metal constituent of the bath capable of reducing sulfids of other metals and also withdrawing partially refined sulfids at the other end of said bath, but at different levels.

In testimony that I claim the foregoing as my invention, I have signed my name in 95 presence of two subscribing witnesses.

NOAK VICTOR HYBINETTE.

Witnesses:

M. E. GUTTORENSEN,  
C. F. HANSEN.